

## UNITED STATES PATENT OFFICE

EDGAR W. FIELDING, OF WILMINGTON, DELAWARE, ASSIGNOR TO E. I. DU PONT DE NEMOURS & COMPANY, OF WILMINGTON, DELAWARE, A CORPORATION OF DELAWARE

## METHOD OF INHIBITING THE OXIDATION AND HYDRATION OF LEAD ALLOYS

No Drawing.

Application filed March 28, 1931. Serial No. 526,142.

This invention relates to a method of preventing the oxidation and hydration of lead-sodium alloys, and particularly to such alloys intended for use in the manufacture of tetra-alkyl-lead.

It has heretofore been the practice in making alloys of lead and sodium to discharge such alloys from the melting pots in which they are made into suitable receptacles holding approximately 500 pounds of alloy, and in which the alloy is cooled. The practice of discharging material in this manner, however, is accompanied by certain disadvantages in that considerable oxidation and hydration occurs, both while the stream of molten alloy is flowing from the alloy pot into the mold, as well as on the surface of the mold during the cooling period. Such a condition tends to destroy the value of lead-sodium alloy when it is employed for certain subsequent purposes, and particularly for the production of tetra-alkyl-lead, and especially tetra-ethyl-lead, or other organo lead derivatives.

An object of the present invention is to overcome the oxidation and hydration of molten lead sodium alloys. A further object is to improve generally upon the condition of lead alloys. Other objects will appear hereinafter.

These objects are accomplished by the following invention in which I have found that the oxidation and hydration of lead sodium alloys can be overcome by the addition of a small quantity of mineral oil to the alloy mold prior to the casting of the charge from the alloy pot. While the quantity and character of the oil may vary within rather wide limits, I preferably add approximately one pint of a high-flash mineral oil. The beneficial effect to be derived from the use of such an oil appears to reside in the fact that when the hot alloy strikes the oil as the alloy flows into the bottom of the mold, part of the oil is vaporized and surrounds the stream of

molten alloy, thus providing a reducing atmosphere which tends to blanket the stream of hot alloy from contact with the air. When the mold is full the oil floats on the surface of the mold and covers the alloy with a protective film.

Other methods of producing an atmosphere of the vapors of the oil will be apparent but I have found the foregoing to be convenient and satisfactory.

I have found that this procedure results in a very material advantage, in that little or no reaction with air occurs during the casting and cooling period, and as a result higher yields of tetra-alkyl-lead, and particularly tetra-ethyl-lead, may be obtained when the alloy is used for the purpose of producing tetra-ethyl-lead by reaction with ethyl chloride or other organo derivatives by reaction with alkyl or aryl halides.

With the view of more clearly defining my invention the following illustrative example of one embodiment thereof is given, but it is to be understood that the scope of my invention is to be limited only as indicated by the patent claims appearing hereinafter:

*Example:*—A lead sodium alloy is prepared in a regulation alloy pot in the usual manner known in the art. When this alloy has been prepared it is cast into cones having a capacity of approximately 500 pounds and which have been previously treated by the addition of one pint of summer black oil such as is used for the lubrication of the journal boxes on railway cars. When the alloy has been cast, it is set aside to cool and solidify.

Other oils which have high flash points, and especially those having flash points above 300° C. may be used for this purpose.

I claim:

1. The process of inhibiting the oxidation and hydration of a hot lead sodium alloy which comprises maintaining an atmosphere of the vapors of a mineral oil having a flash point above 300° C. in contact with the alloy.

2. The process of inhibiting the oxidation and hydration of a hot lead sodium alloy which comprises enveloping the alloy in an atmosphere of the vapors of a mineral oil having a flash point above 300° C.
- 5 3. In the molding of lead alloys, the method of inhibiting the oxidation and hydration of the hot alloys which comprises saturating the inner surfaces of the mold with a mineral oil having a flash point above 300° C. and which will vaporize at least partially at the melting temperature of the alloy.
- 10 4. The method of molding lead alloys and simultaneously inhibiting oxidation and hydration thereof which comprises pouring molten alloy into a mold containing a mineral oil having a flash point above 300° C. and vaporizing at least partially at the melting temperature of the alloy, the oil being in sufficient amount to form vapors enveloping the stream of alloy during the pouring and to form an oil layer above the casting when the mold is filled.
- 15 5. The method of molding lead alloys and simultaneously inhibiting oxidation and hydration thereof which comprises pouring molten alloy into a mold containing summer black oil sufficient in amount to form vapors enveloping the stream of alloy during the pouring and to form an oil layer on the top of the casting when the mold is filled.
- 20
- 25
- 30

In testimony whereof I affix my signature.  
EDGAR W. FIELDING.

35

40

45

50

55

60

65